

## UNITED STATES PATENT OFFICE.

HENRY V. DUNHAM, OF BAINBRIDGE, NEW YORK, ASSIGNOR TO VAN TASSEL COMPANY, OF BOSTON, MASSACHUSETTS, A CORPORATION OF MASSACHUSETTS.

## WATERPROOFING LEATHER.

No Drawing.

Application filed July 6, 1926. Serial No. 120,877.

The present invention relates to the waterproofing of leather and has special reference to waterproofing sole leather or belt leather and other relatively heavy leather but is 5 also applicable to thin leather, split leather, etc. The process has given particularly favorable results in the waterproofing of chrome leather, under which expression is intended to be included, leather tanned or tawed by 10 means of chromium compounds either used alone or in conjunction with vegetable tanning materials. As a special example of this, "chrome-tanned bark-retanned" leather, when treated in accordance with the present 15 invention gives especially favorable results, notably for shoe soles. All chrome tanned leather is particularly good as regards wearing properties, for sole leather and the like. However, it is too stiff for 20 many purposes. It also has the objectionable property of absorbing a large amount of water and when in a wet condition it stretches badly and is very slippery. These 25 disadvantages are overcome by my process as described below in which the leather, besides being made waterproof, becomes pliable and non-slippery and the undesired properties above noted are eliminated.

In accordance with the present invention 30 I impregnate leather, particularly of the kind above referred to, with a mixture consisting of a low-viscosity solution of rubber in a wax, say paraffin wax, to which may be added other substances, which are normally 35 solid or semi-solid such as greases, other gums and resins, drying oils in small amount, dyes, etc. However, it is not desirable to employ volatile solvents in the impregnation. Volatile solvents have heretofore been extensively 40 used in the impregnation of leather and other materials with mixtures including paraffin wax, gums or the like, but the use of these solvents is open to serious objection on account of their inflammability and 45 consequent fire risk. Moreover the volatile solvent absorbed during the impregnation subsequently evaporates, with the result that the materials dissolved therein are largely drawn to the surface of the leather leaving 50 only a very small amount of the impregnating agent in the interior of the leather. Thus the treated leather of such old processes is not sufficiently filled with the rubber and wax and other substances, to possess the 55 desired waterproof qualities.

In accordance with the present invention I preferably use a mixture composed largely or entirely of paraffin wax and rubber. The paraffin is first heated to a temperature substantially above the melting point of the 60 paraffin, and at well above the softening point of rubber, say 150° C., and the rubber, preferably in comminuted form, is then gradually added to the hot material preferably with stirring while preferably at about 65 150° C., or a little higher. Obviously temperatures high enough to ruin the mixture or to distill off the paraffin, or to wholly decompose the rubber, should not be used. The stirring is continued until a uniform smooth 70 mixture is obtained. In this way a product containing, if desired, from 5% up to 50% or more of rubber can be prepared. I preferably use 5% or more of rubber in all cases, 10 to 20% being generally most suitable. In 75 connection therewith I can also add other gums or resins, such as gums thus, gum sandarac, gum yucca, common rosin or the cumarone resins, and also other waxes, such as japan wax, Montan wax, etc. I can also 80 employ with the paraffin and rubber, with or without the other ingredients above referred to, non-volatile drying oils such as linseed oil, tung oil, etc. The materials mentioned in the last two sentences are all organic materials 85 capable of blending with the mixture of rubber and paraffin wax.

In impregnating the leather, the mixture is melted and maintained at a temperature of 90° to 100° C. (preferably 95 to 98° C.) 90 at which temperature the leather is immersed in the molten mixture and allowed to remain for a time depending upon the degree of impregnation desired, the dryness, thickness, hardness and porosity of the leather 95 and other factors. The pieces of leather can be placed in a vertical or horizontal position in the tank containing the hot molten impregnating material. The material should be used sufficiently hot to be molten, but temperatures substantially above 100° C., should generally be avoided as liable to injure the leather. Generally the higher temperatures above given are preferable as the impregnation is very much more rapid at 95 to 98° 100 C., than say at 75 to 80° C. At the lower temperatures the impregnating liquid is much more viscous and has less penetrating power. While I do not desire to limit this invention to the use of these preferred spe- 110

specific temperatures, I call attention to the fact that the leather is immersed in a relatively hot mixture, the same being, for instance, hot enough to injure a person's hands if held therein for any substantial time. This invention is thereby sharply differentiated from greasing boots by applying a soft grease at, or slightly above room temperature.

10 The impregnating mixture which I employ most advantageously is, at normal room temperature, a relatively firm solid, usually of a hardness comparable with some of the softer varieties of crystallizable paraffin 15 wax, scale wax, etc., and is not a soft-greasy mass of the consistency of chicken grease, goose grease, petroleum etc., commonly used for greasing boots.

I call attention to the fact that the mixture of rubber and paraffin wax is heated preferably to 150° C., or thereabout, or to a somewhat higher temperature, during the making of the impregnating medium. I am aware of British patent to Abel, Number 25 1,962 of 1865, in which is described impregnating leather with mixtures of gums (including rubber) and waxes (including paraffin wax) the same having been heated to from 220° F. to 240° F., care being taken 30 not to heat the mixture to over 260° F. Such an impregnating mixture is however, if containing 15% of rubber, of such high viscosity as to be practically useless for impregnating leather at 90 to 100° C. This 35 same mixture however, when heated to 150° C., is of very much lower viscosity. As an illustration, a mixture of 15% rubber and 85% hard paraffin wax, heated to 260° F. (126.7° C.) had a viscosity at 95° C., of 7,000 40 seconds on the Story viscosimeter, while a precisely similar mixture (15:85) heated to 150° C., under precisely similar conditions, had a viscosity of about 480 seconds at 95° C. By heating to over 150° C., the viscosity 45 is somewhat further reduced. Other mixtures (i. e. mixtures of rubber and paraffin in other proportions) heated to about 150° C., or a little below, having a viscosity not substantially above 500 seconds, are also 50 very useful. Obviously the temperature should not be carried to such a high point as to injure the waterproofing qualities of the mixture. The viscosity of the mixture whether heated to 126.7 and 150° C., will be 55 largely dependent upon the rubber content. It is obvious that the permeating qualities of the mixture (at a given temperature) will increase with decreasing viscosity and vice versa.

60 The leather to be impregnated can be soaked in the hot molten mixture, until sufficiently impregnated, this being done at say, 90 to 100° C., preferably 95 to 98° C., say at atmospheric pressure.

65 In impregnating leather for shoe soles,

the leather can be soaked in the waterproofing mixture until sufficiently impregnated, say for about 4 to 6 hours, a heavy belt leather may require 8 hours. This can be hastened by vacuum and pressure treatment, but is generally not needed. The impregnation is for many purposes, carried out as completely as possible, but in some cases a partial impregnation is sufficient.

The leather is preferably quite dry before immersing in the impregnating liquid. I may use air-dried leather but it appears better to further dry the leather in a steam jacketed oven, at say 98-100° C., just before impregnating.

As specific example of the composition to be employed for the impregnating bath the following are given:

*Example 1.*

800 pounds of paraffin wax are melted and then heated at about 150° C., with 200 pounds of Para rubber, with stirring, until a uniform mixture is obtained. Leather is then soaked therein, as above described, at 95° C.

*Example 2.*

2,000 pounds of crude plantation rubber are mixed with 7,800 pounds of paraffin wax and 200 pounds of gum thus added, at 150° C. to 155° C., which temperature is maintained 2½ hours while stirring.

*Example 3.*

8,500 pounds of paraffin wax, 1,000 pounds of vulcanized rubber scrap, and 500 pounds of linseed oil are thoroughly stirred together, at 150° C., for three hours.

While I have herein described a good mode of reducing the viscosity and increasing the penetrating quality of the impregnating agent, this invention is not restricted to such method, but I consider the use of any like mixture of the substances herein described, having the low viscosity and high impregnating or permeating qualities, as within the scope of my invention, irrespective of how such properties are imparted thereto.

The present case is in part a continuation of, and is a substitute for my copending application Serial No. 574,294 filed July 11, 1922.

In the appended claims, the expression "chrome-tanned leather" is intended to cover leather that has been tanned by the use of chromium compounds, either alone or with other tanning agents, such as vegetable tanning agents.

Without limiting myself to the specific examples given by way of illustration, what I claim is:—

1. A method of waterproofing leather which comprises thoroughly incorporating

between 5% and 50% of rubber with molten paraffin wax at about 150° C., until a uniform smooth mixture is obtained, which mixture, if cooled to room temperature is a firm waxy solid, and thereafter impregnating the leather with said mixture, in the absence of volatile solvents, while such mixture is in a hot molten state.

2. A method of waterproofing leather which comprises impregnating the leather with a hot molten mixture, which is a firm solid at room temperature and which contains from 10 to 50% of rubber in molten paraffin wax, together with a substance of a resinous character, such mixture being free from volatile solvents, and such mixture at 90 to 100° C. being of sufficiently low viscosity to readily and thoroughly penetrate thick leather, the amount of such paraffin wax and added substance being sufficient to give the mixture a firm waxy consistency at ordinary room temperature.

3. A method of waterproofing leather which comprises impregnating the leather with a hot molten mixture containing from 10 to 50% of rubber in molten paraffin wax, together with a resinous substance and a drying oil, such mixture being free from volatile solvents and such mixture at 90 to 100° C. being of sufficiently low viscosity to readily and thoroughly penetrate thick leather, and the proportion of paraffin wax and resinous substance being sufficient to give the mixture a firm solid consistency at ordinary room temperature.

4. A method of waterproofing leather which comprises thoroughly incorporating between 5% and 50% of rubber with molten paraffin wax at about 150° C., until a uniform smooth mixture is obtained, which mixture, if cooled to room temperature is a firm waxy solid, and incorporating other water-insoluble organic material capable of readily blending therewith, at any stage of the operation, and thereafter impregnating the leather with said mixture, in the absence of volatile solvents, while such mixture is in a hot molten state.

5. A method of waterproofing leather which comprises thoroughly incorporating between 5% and 50% of rubber with molten paraffin wax at about 150° C., until a uniform smooth mixture is obtained, which mixture, if cooled to room temperature is a firm waxy solid, and thereafter impregnating leather containing chromium compounds with said mixture, in the absence of volatile solvents, while such mixture is in a hot molten state.

6. Leather impregnated with a mixture which is a firm waxy solid at normal temperature, such mixture containing about 78 to 85% of paraffin wax and about 10 to 20% of rubber dissolved therein, such mixture

having been heated to at least 150° C., to 65 impart the desired penetrating properties thereto.

7. A method of waterproofing leather which comprises impregnating leather with a hot molten mixture containing about 78 to 85% of paraffin wax, and at least about 10% of rubber dissolved therein, such mixture having been heated to about 150° C., to 75 impart the desired readily penetrating property thereto.

8. Flexible, substantially non-slippery chrome-tanned leather impregnated with a mixture which is a relatively firm somewhat flexible solid at normal room temperature, but which is liquid when hot, such mixture comprising paraffin wax and from 5 to 50% of a water-proof rubbery gum dissolved therein, such mixture, when hot, having a readily penetrating quality and a low viscosity such as can be imparted thereto by 85 heating a mixture of said substances to 150° C.

9. Leather impregnated with a mixture which is a firm waxy solid at normal temperature, such mixture containing about 78 to 85% of paraffin wax and about 10 to 20% of rubber dissolved therein, such mixture having a low viscosity and a high penetrating power such as can be imparted by heating a mixture of said substances to at least 95 150° C.

10. A method of waterproofing leather which comprises thoroughly incorporating between 5% and 50% of rubber with molten paraffin wax, such operation involving heating such substances to not below 150° C., but not high enough to distill off the wax or spoil the rubber until a uniform smooth mixture is obtained, which mixture, if cooled to room temperature is a firm waxy solid, and thereafter impregnating the leather with said mixture, in the absence of volatile solvents, while such mixture is in a hot molten state.

11. A process which comprises impregnating leather with a hot mixture which at normal room temperature is a firm waxy solid, and which at 95° C. has a viscosity not substantially above 500 seconds (Story), and which mixture contains paraffin wax 110 and a water-insoluble gum.

12. An impregnating and waterproofing agent suitable for impregnating leather which mixture at normal room temperature is a firm waxy solid, and which at 95° C. 120 has a viscosity not substantially above 500 seconds (Story), and which mixture contains paraffin wax and rubber.

13. A rubber-paraffin mixture having viscosity at 95° C., not above 480 seconds 125 (Story) and containing about 15% of rubber.

14. A rubber-paraffin mixture having a low

viscosity when hot, corresponding to that obtained by heating a mixture of said ingredients to at least 150° C.

15. A method of treating leather which comprises impregnating same with a mixture of paraffin wax and rubber, having a low viscosity and a high penetrating power such as can be imparted by heating such mixture to about 150° C.

16. Leather impregnated with a mixture of paraffin wax and rubber, having a low viscosity and a high penetrating power such as can be imparted by heating such mixture to about 150° C.

17. Chrome-tanned bark-retanned leather 15 impregnated with a mixture of paraffin wax and rubber, having a low viscosity and a high penetrating power such as can be imparted by heating such mixture to about 150° C.

18. Chrome-tanned bark-retanned leather impregnated with a low viscosity mixture containing paraffin wax and rubber.

19. A chrome-tanned leather impregnated with a low viscosity mixture containing paraffin wax and rubber.

In testimony whereof I affix my signature.

HENRY V. DUNHAM.